

April 8, 1924.

1,489,790

H. G. SCHANCHE

PROCESS OF MUFFLING LITHOPONE AND APPARATUS THEREFOR

Filed May 11, 1921



Fig. 1



Inventor H. G. Schanche,

By his attorney J. H. Squair.

## UNITED STATES PATENT OFFICE.

HERMAN G. SCHANCHE, OF PHILADELPHIA, PENNSYLVANIA, ASSIGNOR TO E. I. DU PONT DE NEMOURS & COMPANY, OF WILMINGTON, DELAWARE, A CORPORATION OF DELAWARE.

## PROCESS OF MUFFLING LITHOPONE AND APPARATUS THEREFOR.

Application filed May 11, 1921. Serial No. 463,788.

To all whom it may concern:

Be it known that I, HERMAN G. SCHANCHE, a citizen of the United States, and a resident of Philadelphia, in the county of Philadelphia and State of Pennsylvania, have invented a certain new and useful Process of Muffling Lithopone and Apparatus Therefor, of which the following is a specification.

10 This invention relates to the manufacture of lithopone and more particularly it relates to a process of muffling lithopone and to apparatus wherewith such process may be readily and conveniently carried out.

15 In the manufacture of lithopone, one of the important steps is the calcination of the pigment. The precipitated mixture of zinc sulphide and barium sulphate, ordinarily known as raw lithopone, is filtered and at 20 least partially dried, and then heated until it is perceptibly red (the color first appears below 600° C.). After the proper temperature has been reached the pigment is quenched in water. By the calcination the tinting

25 strength of the pigment is increased and the oil absorption is decreased. At intervals during the above mentioned calcination the lithopone is customarily stirred or rabbled with rakes operated by hand; this operation 30 is not only burdensome, but makes it difficult to avoid excessive oxidation of the lithopone by air which gains entrance while the stirring is being performed. I have devised a process and apparatus for calcining lithopone whereby these objections may be overcome, and a high grade lithopone obtained.

In brief, the invention consists in calcining the lithopone while preventing access of air thereto at any time during the calcination, and in apparatus therefor. By working in accordance with the invention, excessive oxidation of the pigment during calcination is eliminated and pigment of desired character is readily produced.

45 Some of the literature on lithopone, of course, refers to calcination in "sealed retorts" or "with exclusion of air," although the reason for the precaution is not given. Obviously however, these terms are used in 50 but a comparative sense, to make plain that the operation is not one of roasting, and that the doors of the lithopone muffles are kept closed as much as possible. In actual working the lithopone is shoveled into the fur-

nace, of course with the doors open; it is rabbled, again of course with the doors open to permit introduction of the rabbled tool; and finally it is raked out for quenching, yet again with the doors open. In the sense of the present invention this is not working with exclusion of air; it cannot prevent the development of the yellowish tint which is characteristic of a lithopone that is "off color."

65 In describing my invention in detail, I shall first describe the illustrated furnace embodying it so far as it relates to apparatus, but although I describe the invention by reference to such illustrated apparatus it will be understood that I do not restrict it thereto. In the accompanying drawings of this furnace:—

70 Figure 1 is a cross-sectional view substantially on the line 1—1 of Figure 2, looking in the direction of the arrows, with certain parts broken away to economize space;

75 Figure 2 is a top plan view to a somewhat smaller scale than Figure 1, and

80 Figure 3 is a top plan view of one of the air-excluding feeders.

The illustrated furnace comprises in general a fire box 1 having a suitable grate 1<sup>a</sup>, and a calcining structure 2 or muffle. The latter includes, a hearth structure in the form of an upper hearth element 3 and a lower hearth element 4, domed partitions 5 and 6 providing the annular chamber 7 in communication with the fire box 1, by the passage 8 entering at 9, to directly receive the flue gases therefrom, and the annular chamber 10 below the lower hearth element 4. The chamber 7 is connected with the chamber 10 by the flue 11, and the chamber 10 is connected with the stack 12 by the flue 13. A baffle wall 14 located between the entrance 9 and the flue 11 closes the chamber 7, and a baffle wall 15 closes the chamber 10 between the flues 11 and 13. With this construction, the flue gases enter at 9, travel anti-clockwise (Fig. 2) around the chamber 7, pass down the flue 11, travel anti-clockwise around the chamber 10, and pass into the stack 12 at 13; thus the hearth structure is heated, the lower element to a higher temperature than the upper.

100 The walls of the furnace structure are air-excluding. As here shown, the side walls are composed of steel *s* asbestos *a*, red brick

85

90

70

75

80

85

90

95

100

105

b and fire brick c. The top 17, partitions 5 and 6, walls 14 and 15, and bottom 18, are of fire brick. The hearth structure may be of any suitable material, as tile. To provide 5 for the escape of steam from the wet raw lithopone, an escape pipe 40 is provided in the top 17; when working there is sufficient excess pressure in the calcining structure to substantially ensure that no air will enter 10 through the pipe. Desirably the hearth elements are supported by struts 5<sup>b</sup> and 18<sup>a</sup>.

In further accordance with the invention, a shaft 16, desirably hollow for cooling, is centrally and rotatably borne in the top 17 15 and bottom 18 in such manner as to exclude air, as by the close fitting bearings 17<sup>a</sup> and 18<sup>a</sup>. This shaft carries two diametrically extending arms 19 and 20, one in each chamber 3<sup>a</sup> or 4<sup>a</sup>. On each arm is carried a series of 20 plows or agitating devices 19<sup>a</sup> or 20<sup>a</sup>. Each plow is in the character of a vertical plate 21, connected with the related arm at 22. The plates are set with their vertical planes at an angle to the radii of the hearth element, the plates for the upper element being set to move the material on the hearth radially inward, and those for the lower being set to move the material outward, as the shaft 16 rotates. The hearth elements 25 are connected for the fall of material from the upper to the lower by the passage 23 formed by the upstanding circular extensions 5<sup>a</sup> and 6<sup>a</sup> of the partitions 5 and 6. With the construction outlined it will be 30 seen that lithopone can be continuously moved through the furnace (traveling gradually around and across the hearth elements) and while being thus moved through the furnace will be continuously stirred and 35 agitated, the operation being carried on with exclusion of air, the access of air which is a necessary accompaniment of rabbling in the ordinary manner being eliminated.

In yet further accordance with the invention, means are provided for the feeding of the lithopone to the furnace, and the feeding of it from, i. e., discharging of it from, the furnace, with the exclusion of air. As here illustrated such means comprises a 45 feeder 24 at the top of the furnace and in communication with the hearth element 3, adjacent its periphery, by the passage 25, and a similar feeder or discharger 26 in communication with the periphery of the hearth 50 element 4 by the downwardly sloping passage 27. Each device comprises a cylindrical casing 28 in which is axially and rotatably mounted a feeder proper 29 comprising a series of blades 30 radiating from the rotatable shaft 31. These blades are sufficient 55 in number to provide that they shall at all times close the passage 25, or 27; the blades fit closely in the casing 28 and travel close to the walls thereof, and the device is tightly 60 connected with the furnace walls. Thus the 65

lithopone can be fed to and taken from the furnace without access of air.

Desirably the shaft 31 of each device is continuously driven, as by the wheel 32 being connected to any suitable driving means 70 as an electric motor (not shown.) The wheel 32 of each device is connected to the related shaft 31, preferably by reduction gearing 33. The central shaft 16 is continuously driven, as from an electric motor 75 (not shown) connected to the wheel 34 geared with the lower end of the shaft 16 by the reduction gearing 35, 36, 37, 38, 39.

The arrangement provides for the continuous calcination of lithopone since the material can be continuously fed in at the device 24, continuously moved across the hearth 3-4, and continuously discharged through the device 26, and the entire calcining operation is performed without access 80 of air, as neither the feeders nor the stirrer appreciably permit air to enter the furnace. 85

The general method of carrying on the process with the aid of the furnace will be evident from the above description. As to certain details of operation: the upper hearth element is preferably heated (by radiation) to somewhat above 250° C. and the lower to about 550° C. to 750° C.; the shaft 16 is driven at a speed to provide that a given portion of the lithopone passing through the furnace will be raised to, and maintained at, a temperature ranging between 550° and 750° C. long enough (for example 1 hour at 650° C.) to impart the desired hiding power by the time said portion reaches the passage 27, and the devices 24 and 26 are driven at a speed to supply and remove the lithopone at a rate to ensure continuous uninterrupted operation. The lithopone discharged at 26 is quenched in 90 water contained in the trough 41.

In applying the terms "air excluding" and the like to the various structures above mentioned, I mean to include structures which although not absolutely air tight yet exclude air to such an extent that the amount of air which does enter is insufficient to render the lithopone off color, that is, insufficient to reduce the brightness or deepen 110 the tint of the lithopone to an objectionable extent for paint purposes. For example, when calcining lithopone comprising a small amount of chlorides absolute exclusion of air is not essential, although such a degree of exclusion as will prevent discoloration, and by reason of that can properly be called "air exclusion" in contradistinction to the haphazard methods of the prior art, is essential; and a furnace which would exclude such air as would be harmful when working with such chloride-containing lithopone, although perhaps not excluding all air, would be air-excluding and fall within my invention, and the calcining operation would be, to all 115 120 125 130

intents and purposes, carried on while preventing access of air.

If desired, a suitable baffle-wall-and-flue arrangement for conducting the gases from the chamber 10 and around the space between the upper hearth element 3 and the partition 5 in their travel to the stack 12 may be provided.

As will be understood by those skilled in the furnace building art, such flues for bypassing the gases directly to the stack, dampers, and so on, as are desirable for convenience in controlling the temperature may be provided, also, although I have referred to the chambers, as 7, as receiving "flue gases", of course as is usual in muffle furnaces combustion need not be confined to the fire box.

I claim:—

1. The process of muffling lithopone which comprises agitating the lithopone during calcination thereof while preventing access of air thereto.

2. The process of muffling lithopone which comprises calcining lithopone at a temperature of from about 600 to 700° C. while excluding air therefrom, and frequently stirring said lithopone during calcination while maintaining said exclusion of air.

3. The process of muffling lithopone which comprises passing a stream of lithopone, while agitating the same, through a calcining zone from which air is excluded, and heating the lithopone passing through said zone to a temperature of from about 600 to 700° C.

4. The process of making lithopone which comprises continuously passing a stream of lithopone first through a calcining zone maintained at a temperature of from about 600 to 700° C. and then into a quenching liquid.

5. The process of muffling crude lithopone which comprises continuously passing a stream of lithopone, while stirring the same to secure uniform heating thereof, through a zone maintained at a calcining temperature.

6. The process of muffling crude lithopone containing a small proportion of a chloride which comprises continuously passing a stream of said lithopone through a calcining zone maintained at a temperature sufficiently high to give the lithopone the desired strength while stirring the lithopone and while preventing access to the lithopone in the calcining zone of air in an amount sufficient to cause the resulting finished lithopone to be off color.

7. The process of muffling crude lithopone containing a chloride which comprises continuously passing a stream of said lithopone through a calcining zone while preventing access to the lithopone in the calcining zone of air in an amount sufficient to reduce the brightness or deepen the tint of the litho-

pone to an objectionable extent for paint purposes.

8. A muffle furnace for calcining lithopone comprising a calcining structure of air-excluding character and including a hearth structure, and agitating means having an air-excluding mounting in said calcining structure and associated with said hearth structure to agitate the lithopone thereon. 70

9. A muffle furnace for calcining lithopone comprising a calcining structure of air-excluding character and including a hearth structure, an air-excluding feeding device located to discharge lithopone upon said hearth structure, and an air-excluding discharging device located to discharge lithopone from said hearth structure. 80

10. A muffle furnace for calcining lithopone comprising a calcining structure of air-excluding character and including a hearth structure, an air-excluding feeding device located to discharge lithopone upon said hearth structure, an air-excluding discharging device located to discharge lithopone from said hearth structure, and movable 90 transferring means having an air-excluding mounting in said calcining structure and located in proximity to said hearth structure for moving lithopone on said structure from adjacent said feeding device to said discharging device. 95

11. A muffle furnace for continuously calcining lithopone comprising a calcining structure of air-excluding character and including a hearth structure, a continuously 100 operable air-excluding feeding device located to discharge lithopone upon said hearth structure, a continuously operable air-excluding discharging device located to discharge lithopone from said hearth structure, continuously operable movable transferring means having an air-excluding mounting in said calcining structure and located in proximity to said hearth structure 105 for moving lithopone on said structure from adjacent said feeding device to said discharging device and means for driving said two devices and said transferring means. 110

12. A muffle furnace for calcining lithopone comprising a calcining structure of 115 air-excluding character and including hearth structure presenting an upper and a lower hearth element and a passage therebetween for the fall of lithopone from the upper to the lower element, and movable transferring means having an air-excluding mounting in said calcining structure and including provisions for moving lithopone across said upper hearth element and to said passage. 120

13. A muffle furnace for calcining lithopone comprising a calcining structure of air-excluding character and including a hearth structure presenting an upper and a lower hearth element and a passage therebetween for the fall of lithopone from the upper to 125 130

- the lower element, an air-excluding feeding device located to discharge lithopone upon said upper element and spaced from said passage, an air-excluding discharging device located to discharge lithopone from said lower element and spaced from said passage, and movable transferring means having an air-excluding mounting in said calcining structure and including provisions for moving lithopone from adjacent said feeding device across said upper element to said passage, and for moving lithopone from adjacent said passage across said lower element to said discharging device.
14. A muffle furnace for calcining lithopone comprising a calcining structure of air-excluding character and including a hearth structure presenting an upper and a lower

hearth element, each substantially circular, and a central passage therebetween for the fall of lithopone from the upper to the lower element, an air-excluding feeding device located to discharge lithopone upon said upper element near its periphery, an air-excluding discharging device located to receive lithopone from adjacent the periphery of the lower element, and transferring means comprising a rotatable shaft having an air-excluding mounting in said calcining structure and carrying devices for moving lithopones around and radially inward on said upper element and around and radially outward upon said lower element, upon rotation of said shaft.

In testimony whereof I affix my signature.  
HERMAN G. SCHANCHE.